

June 12, 1973

MAKOTO YOSHIDA ET AL  
COLOR PHOTOGRAPHIC LIGHT-SENSITIVE MATERIALS FOR A SILVER  
DYE BLEACHING PROCESS  
Filed Oct. 19, 1970

3,738,839



INVENTORS  
MAKOTO YOSHIDA  
SHINICHI IMAI  
JUNIJI TAMANO

BY *Sughrue, Rothwell, Muon,*  
*Zinn & Macpeak*  
ATTORNEYS

# United States Patent Office

3,738,839  
Patented June 12, 1973

## 1

3,738,839

### COLOR PHOTOGRAPHIC LIGHT-SENSITIVE MATERIALS FOR A SILVER DYE BLEACHING PROCESS

Makoto Yoshida, Shinichi Imai, and Juniti Tamano, Kanagawa, Japan, assignors to Fuji Photo Film Co., Ltd., Kanagawa, Japan

Filed Oct. 19, 1970, Ser. No. 82,033  
Int. Cl. G03c 1/10

U.S. Cl. 96—99

6 Claims

#### ABSTRACT OF THE DISCLOSURE

A color photographic light-sensitive material for a silver dye bleaching process comprising a support having thereon a photographic emulsion layer containing a cyan dye represented by the following general formula:



wherein said nitro group is at the para- or meta-position of the benzoyl nucleus and method for preparing same is disclosed.

## 2

certain properties, such as stability to the severe development, dye bleaching treatment, and silver bleaching treatment in a silver dye bleaching process. In addition, the dye should have sufficient fastness to light, heat and humidity.

#### SUMMARY OF THE INVENTION

It, therefore, is an object of the present invention to provide color photographic light-sensitive materials containing an excellent novel cyan dye which satisfies the above-mentioned criteria.

Still, it is another object of the present invention to provide dyes which are easily produced and excellent in color and hue.

These and other objects are attained by using a cyan



#### BACKGROUND OF THE INVENTION

The present invention is concerned with a color photographic light-sensitive material for a silver dye bleaching process, said light-sensitive material containing a specific cyan dye in the silver halide light-sensitive emulsion layer thereof.

Many of cyan dyes for color photographic light-sensitive materials applicable to silver dye bleaching processes are azo dyes and it is necessary that these azo dyes be bleached in proportion to the silver image formed by development in order to provide a cyan colored positive image. Accordingly, in order that a dye of this nature can be used, the azo group present in the dye must be readily decomposed by reduction in proportion to the amount of silver present so as to permit the dye to be completely bleached. Furthermore, it is necessary that in cases where the dye is to be incorporated into a silver halide emulsion layer, that the dye not diffuse into other emulsion layers and diminish photographic properties such as fog and desensitization. Moreover, the dye must maintain

55 wherein the nitro group may be in the para-position or the meta-position on the benzoyl nucleus.

The cyan dyes used for color photographic light-sensitive materials applicable to the silver dye bleaching process are mainly bisazo dyes. According to a general method for producing those bisazo dyes, 4-nitro-2,5-dimethoxyaniline is first diazotized and coupled with 1-amino-8-naphthol-3,4-disulfonate derivative to provide a monoazo-nitro compound. The product so obtained is reduced to give a monoazoamino compound, and this amino compound is diazotized and coupled with a 1-amino-8-naphthol-3,4-disulfonate derivative to provide the bisazo dye.

The above reaction is usually conducted in a aqueous solution. However, since the intermediate products prepared in the above reaction and the dye are easily soluble in water, a large amount of a salt must be added to the reaction system to salt out the final product from the reaction product liquid. Moreover, it is quite difficult to obtain the pure dye by removing salts contained in the dye thus salted out. Hence, in the case of producing a dye which is too easily soluble in water, the production proc-

ess becomes hampered and the yield of the dye is reduced. This results in higher dye cost as well as the dye remaining unsuitable for color photographic light-sensitive materials.

#### DETAILED DESCRIPTION OF THE INVENTION

Therefore, the inventors have investigated dyes which can be produced with a good yield by a simple production process and yet provide dyes which are suitable for purposes of the present invention. The dyes used in this invention have one nitro group at the para-position or the meta-position of the benzoyl nucleus. The solubility of the dye in water is low as compared with that of dye A having no nitro group and shown by the following formula:

Dye A



Upon comparing the diffusion coefficient of the dyes in gelatin as a comparison for showing their solubility in water, the diffusion coefficients of the dyes represented by the above-mentioned general Formula I having a nitro group at the para-position or the meta-position are  $0.02 \times 10^{-8}$  cm.<sup>2</sup>/sec. in both cases. On the other hand, dye A shown above and a dye represented by the general Formula I wherein a nitro group is at the ortho-position have diffusion coefficients of  $0.12 \times 10^{-8}$  cm.<sup>2</sup>/sec. and  $2.2 \times 10^{-8}$  cm.<sup>2</sup>/sec., respectively. Thus, the diffusion coefficient of the dye of this invention is about  $\frac{1}{6}$  of that of the dye A and about  $\frac{1}{10}$  of that of the ortho-nitro substituted dye, which illustrates that the dyes of the present invention are weakly soluble in water. Dye A and the ortho-nitro substituted dye will be diffused from a gelatin layer and hence are unsuitable as dyes for color photographic light-sensitive materials. The above-mentioned excellent property of the dyes of the present invention resides in the effect of the substituted nitro group and the position of the nitro group. It has not been expected that one nitro group and the position of the nitro group could provide such an influence on the solubility of these dyes in water. In addition, the diffusion coefficient of these dyes in gelatin is obtained by measuring the concentration of the dye diffused in pure gelatin when a gelatin gel containing the dye is brought into contact with pure gelatin for a definite period of time. Calculations are then made according to Fick's law.

As mentioned above, since the dyes of the present invention have a desirable low solubility in water, they may be prepared with excellent yield, low cost and can be very profitable as a cyan dye for color photographic light-sensitive materials.

Also, as made clear from the accompanying drawing, the dyes of the present invention give very excellent color and hue as compared with that of an ortho-nitro substituted dye which is a structural isomer.

#### BRIEF DESCRIPTION OF THE DRAWING

That is to say, in the figure of the accompanying drawing, curve 1 stands for the absorption curve of an aqueous solution of a dye of the present invention represented by Structural Formula 1 shown below, curve 2 stands for the absorption curve of an aqueous solution of a dye of the present invention represented by Structural Formula 2, and curve 3 stands for the absorption curve of an aqueous solution of the ortho-nitro substituted dye which is a structural isomer of the dyes of the present invention.

It has been discovered that the color photographic light-sensitive materials produced by using a cyan dye of this invention are excellent in their reflectivity curve and give an ideal cyan color and hue. Therefore, the cyan dyes of the present invention are particularly useful for reflection-type color photographic light-sensitive material.

The cyan dyes of this invention can be effectively incorporated in silver halide photographic emulsion without diminishing the photographic properties thereof. When they are incorporated into a silver halide photographic emulsion layer, they can be easily bleached in proportion to the silver image. The cyan dyes of this invention also possess sufficient fastness to development of chemicals, heat, light and moisture and are thus quite desirable for color photographic light-sensitive material applicable to a silver dye bleaching process.

The cyan dyes of the present invention can not only be used in natural color photographic light-sensitive materials for the silver dye bleaching process but also in color photographic light-sensitive materials for silver dye

15

bleaching process wherein mono-color images and two-color images are desired.

The concentration of the cyan dye is determined by a preliminary test, in order to provide the proper image density. Accordingly, the concentration necessary can be easily determined by the skilled in the art of photographic materials.

The cyan dyes of the present invention are those shown in the following formulae:

The dye portion illustrated as,



is denoted by A;

Formula 1



Formula 2



These dyes may be prepared by a straight forward process as described below: all parts are by weight unless otherwise stated.

#### SYNTHESIS 1.—THE DYE HAVING STRUCTURAL FORMULA 2

##### (1-1): Synthesis of the diazo component

198 parts of 1-amino-2,5-dimethoxy-4-nitrobenzene were diazotized in a suspension of strong hydrochloric acid. This diazotized liquid was added to 423 parts of a solution containing 1-benzoylamino-8-hydroxynaphthalene-3,6-disulfonic acid made alkaline with sodium carbonate to effect coupling. The nitroazo dye thus obtained was reduced in an alkaline solution by sodium sulfide to form the corresponding aminoazo dye, which was then isolated (see, Japanese patent publication No. 25,768/1964).

##### (1-2): Synthesis of the coupling component

40 parts (by volume) of a 30% aqueous sodium hydroxide solution and 400 parts (by volume) of water

70

75

were added to 93 parts of 1-amino-8-naphthol-3,6-disulfonate. After adding 65 parts of sodium carbonate and 72 parts of m-nitrobenzoyl chloride at 35° C., the resultant mixture was heated to 95° C. for 2 hours. During heating, crystal of sodium carbonate was added to the mixture, whereby the mixture was always maintained in a weak alkaline state. After adding to the mixture 100 parts (by volume) of concentrated hydrochloric acid and 200 parts (by volume) of a saturated aqueous solution of sodium chloride, the product was recovered by filtration and dried. The yield of the product was 96 parts.

(1-3): Synthesis of dye (2)

10 parts of the monoazoamino compound obtained in synthesis (1-1) were dissolved in 150 parts of an aqueous solution containing 25 parts of sodium hydroxide. Subsequently, 1.5 parts of sodium nitrite in 10 parts (by volume) of water were added to the solution prepared above. After adding to the mixture 15 parts (by volume) of concentrated hydrochloric acid at 20° C., the resultant mixture was stirred for 1 hour.

8 parts of the coupling component obtained in synthesis (1-2) were dissolved in a solution containing 150 parts (by volume) of pyridine in 75 parts (by volume) of water. The above-prepared diazonium liquid was added dropwise to the solution at 0-5° C. After allowing to stand overnight, sodium chloride was added to the solution and the dye produced was redissolved in water followed by repeating the salting out process until all purple impurities disappeared. Thereafter, the dye formed was salted out by sodium acetate and after recovering the crystals formed by filtration, the crystals were washed with ethanol and dried. The yield was 9.5 parts. The maximum absorption wave length of an aqueous solution of the dye was 613 millimicrons.

SYNTHESIS 2.—THE DYE OF THE STRUCTURAL

The objective dye was produced by repeating the same procedure as Synthesis 1 except that p-nitrobenzoyl chloride was used for the synthesis of the coupling component. The maximum absorption wave length of the aqueous solution of the dye was 620 millimicrons.

A better understanding of the present invention may be obtained from the following examples which are merely intended to be illustrative and not limitative of the present invention. All parts are by weight unless otherwise stated.

EXAMPLE 1

1 part of the cyan dye shown by the Structural Formula 2 was dissolved in 100 parts (by volume) of aqueous sodium hydroxide solution. 80 parts (by volume) of the cyan dye solution was mixed with 100 parts of silver bromide emulsion containing about 30 parts/kg. of silver bromide. The mixture was then applied to a film base.



The light-sensitive film thus obtained was exposed un-

der a step wedge and developed for 10 minutes by a developing liquid having the following composition:

|                                  | Parts |
|----------------------------------|-------|
| N-methyl-p-aminophenol ½ sulfate | 2     |
| Anhydrous sodium sulfite         | 30    |
| Hydroquinone                     | 8     |
| Sodium carbonate                 | 20    |
| Potassium bromide                | 4     |
| Water added to make 1 liter.     |       |

The photographic film thus developed was washed with water and then fixed for 4 minutes by a solution having the following composition:

|                              | Parts |
|------------------------------|-------|
| Anhydrous sodium thiosulfate | 350   |
| Anhydrous sodium sulfite     | 10    |
| Water added to make 1 liter. |       |

The photographic film was then washed with water, hardened by an aqueous solution of 4% formaldehyde, washed with water again, and then processed for 15 minutes by a dye bleaching bath having the following composition:

|                                            | Parts |
|--------------------------------------------|-------|
| Thiourea                                   | 60    |
| Potassium bromide                          | 30    |
| Concentrated hydrochloric acid (by volume) | 30    |
| 2-amino-3-hydroxyphenazine                 | 0.01  |
| Water added to make 1 liter.               |       |

The film was washed with water, fixed again by the fixing bath shown above, washed again with water, and dried.

By these processings, the highlight portion of the photographic film was completely bleached and at the same time a clear cyan image having the absorption maximum at 624 millimicrons was obtained. The cyan image was suitable as a cyan component image for a multi-color light-sensitive material useful in the silver dye bleaching process.

EXAMPLE 2

By repeating the same procedure as in Example 1, using the cyan dye shown by the structural Formula 1, a clear cyan image having the absorption maximum at 623 millimicrons was obtained. The highlight portion of the color image had been completely bleached and hence the cyan image was suitable as a cyan component image for a multi-color light-sensitive material useful in the silver dye bleaching process.

Although the present invention has been adequately described in the foregoing specification and examples included therein, it is readily apparent that various modifications and changes may be made without departing from the scope thereof.

What is claimed is:

1. A color photographic light-sensitive material for a silver dye bleaching process comprising a support having thereon a photographic emulsion layer containing a cyan dye represented by the following general formula:



3. The color photographic light-sensitive material of claim 1 wherein said cyan dye is



4. A method for preparing the color photographic light- 10 sensitive material of claim 1, which comprises:

(a) dissolving a cyan dye of the formula:



wherein said nitro group is at the para- or the meta- 20 position of the benzoyl nucleus in an aqueous alkali metal hydroxide solution.

(b) mixing the solution of (a) with a silver halide emulsion, and

(c) applying the mixture of (b) to a film base.

5. The method of claim 4 wherein the nitro group of 25 the benzoyl nucleus is in the para-position.

6. The method of claim 4 wherein the nitro group of 30 the benzoyl nucleus is in the meta-position.

#### References Cited

#### UNITED STATES PATENTS

|              |         |         |       |       |
|--------------|---------|---------|-------|-------|
| 3,236,643    | 2/1966  | Husek   | ----- | 96-99 |
| 3,287,132    | 12/1966 | Hunt    | ----- | 96-99 |
| 25 3,443,952 | 5/1969  | Anderau | ----- | 96-99 |
| 3,443,953    | 5/1969  | Loeffel | ----- | 96-99 |
| 3,454,402    | 7/1969  | Anderau | ----- | 96-99 |
| 3,454,401    | 7/1969  | Mory    | ----- | 96-99 |
| 3,455,695    | 7/1969  | Piller  | ----- | 96-99 |

J. TRAVIS BROWN, Primary Examiner

E. C. KIMLIN, Assistant Examiner